

Dec. 23, 1941.

E. A. TIPPETTS

2,267,055

PRODUCTION OF REGENERATED CELLULOSE YARN

Filed June 10, 1939



## UNITED STATES PATENT OFFICE

2,267,055

## PRODUCTION OF REGENERATED CELLULOSE YARN

Emerson A. Tippetts, Kenmore, N. Y., assignor to  
 E. I. du Pont de Nemours & Company, Wilmington, Del., a corporation of Delaware

Application June 10, 1939, Serial No. 278,426

2 Claims. (Cl. 18—54)

This invention relates to the production of regenerated cellulose yarn which is composed of extremely fine denier filaments. It relates more particularly to the production of such fine denier filament yarn by an improved process of the type wherein the freshly precipitated regenerated cellulose yarn is subjected to a stretching operation while in contact with a liquid having an elevated temperature.

Heretofore, in the production of fine denier filament yarn by the viscose process it has been commercially uneconomical to produce yarns the filaments of which were finer than about one denier per filament. Furthermore, the previously known processes for the production of such one denier per filament yarns were attended by difficulty of spinning and very material and objectionable yarn degradation.

It is an object of the present invention to produce, by the viscose process, regenerated cellulose yarn composed of filaments having a denier of less than one.

It is another object of this invention to produce, by the viscose process, regenerated cellulose yarn composed of filaments having a denier of the order of 0.5 to 0.75.

It is a further object of the present invention to provide a process for the production of extremely fine denier filament regenerated cellulose yarn from viscose, which process represents an improvement in efficiency and decreased filament degradation over previously known processes.

It is a still further object of the present invention to provide a process for the production of extremely fine denier filament regenerated cellulose yarn from viscose by subjecting the previously regenerated yarn to a stretching operation while in contact with a liquid having an elevated temperature.

Other objects of the invention will appear hereinafter.

In accordance with the present invention, the fine denier filament yarns, which are formed by the extrusion of a viscose solution into a coagulating and regenerating bath under low tension, are passed into a hot (60° C. to boiling temperature) liquid and stretched a sufficient amount to materially reduce the denier thereof while passing through said hot liquid for a distance not to exceed 45 inches based on spinning speeds of at least 3000 and up to 8000 or more inches per minute. Exceedingly gratifying results are obtained when the hot liquid bath is a hot sulfuric acid bath.

It has now been found that regenerated cellu-

lose filaments having a denier of less than one, for example, having a denier of the order of 0.5 to 0.75, can be spun from viscose if the freshly spun filaments, spun under low tension, are removed from the regenerating bath and passed into a stretching bath having a temperature of between 60° C. and the boiling temperature of the bath liquid, in which they are given a material stretch.

It has been discovered that very material advances in economy and material reduction in 10 yarn degradation will be obtained if the freshly precipitated fine denier filament yarns are stretched in a hot sulfuric acid bath, and if the contact with the said hot sulfuric acid bath is 15 confined to a distance of 45 inches or less based on spinning speeds of 3000 to 8000 inches per minute.

On the basis of spinning speeds of the order of 20 3000 to 8000 inches per minute the 45-inch maximum contact of the fine denier filament yarns with hot sulfuric acid during the stretching operation is critical, from a standpoint of yarn degradation, when compared with the prior art processes in which it was considered necessary to 25 contact the threads in hot liquids for a distance of 2 to 12 meters (78 to 460 inches) at speeds considerably less than 3000 inches per minute.

The procedure and apparatus by means of 30 which the process of the present invention may be carried out will be clearly apparent from the following description when taken in connection with the accompanying illustration.

The accompanying illustration is a diagrammatic perspective view of one form of apparatus 35 suitable for use in accordance with the present invention.

Referring to the illustration, reference numeral 11 designates a spinneret which is positioned in tank 13 containing a coagulating and regenerating bath 15. A viscose solution is extruded through spinneret 11 into bath 15 for the formation of a multifilament yarn 17. The yarn 17 is passed about pin 19 which functions as a convergence guide to bring the several extruded filaments together into a single yarn. The yarn is then passed about a plurality of roller guides 21, thence around guide 23. After passing around guide 23 the yarn is drawn from the coagulating and regenerating bath by means of transfer roller 25. The yarn may be looped one or more times 40 about the transfer roller 25 to prevent slippage of the yarn thereon. The yarn is then passed around rollers 33 which are submerged in a hot sulfuric acid bath 29 in tank 27. The yarn is 45 drawn from the hot sulfuric acid bath 29 and

passed onto a collecting bobbin 35. The hot acid bath 29 in tank 27 is maintained at the proper elevated temperature, 60° C. to boiling temperature, in any desired manner, for example, by means of steam coils 31 positioned in the bottom of the tank. The composition of the acid bath 29 may be maintained substantially constant by the continuous, or periodic addition of a replenishing solution of predetermined composition through conduit 37. A portion of the hot acid bath from tank 27 may be continuously or periodically pumped into the coagulating and regenerating bath 15 by means of pump 42 and conduit 39, or the hot acid bath may be drained through conduit 40. Spent coagulating and regenerating liquid may be passed from the coagulating tank 13 through conduit 41.

It is to be understood that the illustrated and above-described apparatus is disclosed for illustrative purposes only. Obviously various different forms and modifications of apparatus can be employed equally well.

The number and type of roller guides 24 in the coagulating and regenerating bath will be determined by the spinning speed, by the size of the threads or filaments being spun, by the tension to be imposed on the yarn, and by the composition of the coagulating and regenerating bath liquid. It is necessary to maintain sufficiently low tension on the yarn during its travel through the regenerating bath to allow sufficient stretch to be imposed thereon during its passage through the hot acid bath so that the desired reduction in yarn denier can be attained. The transfer roller 25 may be made of such size and provided with such a surface that the thread or yarn need not be looped around the same to prevent slippage. On the other hand, the transfer roller may comprise a pair of cooperating squeeze rollers or a pair of spaced rollers about which the yarn is repeatedly passed to prevent yarn slippage and arranged so as to prevent the passing threads from overlapping and chafing each other. The transfer roller may be rotated by the pull exerted thereon by the yarn, or the roller may be positively driven in any desired manner. The collecting bobbin may be of any type well known in the art. The collecting bobbin will, of course, be provided with necessary traverse guides in a manner well known in the art. If desired, the yarn may be drawn through the hot acid bath 29 by means of a feed roll or the like and collected in a rotating bucket in accordance with the conventional bucket process for the production of rayon yarn. In any event, the collecting bobbin, or the feed roller when using the bucket process, will be rotated at a peripheral speed sufficiently higher than the peripheral speed of transfer roller 25 to impart a stretch to the yarn as it passes through the hot acid bath 29. The stretch imposed on the yarn in the bath 29 may be as low as 5% or 10%; however, to obtain the greatest benefit from the present invention the stretch imposed should be 30% to 60% or even 100% or more, depending upon the tension imposed in the spinning bath, upon the physical characteristics to be imparted to the yarn, and limited by the stretch the yarn will stand without breaking.

The spent coagulating and regenerating liquid may be discarded, or it may be renovated, as desired.

For convenience the invention will be described in terms of a spinning process as depicted in the drawing where the yarn is collected on a spin-bobbin.

To avoid confusion the term "spinning speed" will be understood to refer to the peripheral velocity of the spin-bobbin in the bobbin process or the feed wheel speed in the bucket process, and the term "spinning tension" is the tension on the yarn, measured at a point just ahead of the spin-bobbin or its equivalent, when the spinning process is in actual operation.

To further illustrate the principles of the invention, the following examples are given, but it is to be understood that the invention is not necessarily limited thereby. In all of these examples viscose prepared from cotton linters and containing approximately 7% cellulose and 6% sodium hydroxide is used. Obviously viscose having different characteristics can be employed in the practice of the invention depending upon the type of yarn to be produced. Particularly good results have been obtained by the use of a viscose spinning solution which has been ripened to a point where it has an index materially greater than 4.0, for example an index of 4.5 to 6.0, or even greater, as determined by the method of Reinthaler and Rowe, "Artificial Silk," 1928, page 69.

#### Example I

Viscose is passed through a spinneret containing 100 holes, with an average viscose delivery of 7.7 grams per minute, into an aqueous spinning bath containing 9% sulfuric acid, 19% sodium sulfate, 4% glucose and 0.85% zinc sulfate, said bath being maintained at 45° ± 1° C. The extruded filaments are guided through this bath by a plurality of roller guides selected to impose a slight tension on the yarn during a bath travel of 26 inches. The yarn is withdrawn from the bath and passed over a yarn driven transfer roller into a secondary bath which consists of an aqueous solution containing 2% sulfuric acid and which is maintained at a temperature of 90° ± 2° C. The yarn is guided through the secondary bath by a plurality of roller guides selected so that at a spinning speed of 4500 inches per minute the spin tension will be 29 grams when the peripheral speed of the yarn driven transfer roller is 3040 inches per minute. The finished yarn, after washing on the bobbin on which it has been collected, and twister drying in accordance with the method described in Parker and Standley U. S. Patent No. 2,130,247, has a denier of 50 (0.5 denier per filament), a dry tenacity of 3.16 grams per denier and a wet tenacity of 1.8 grams per denier with dry and wet elongations of 8% and 9.3% respectively. After washing and bleaching a high tenacity textile yarn of fine denier is obtained having dry and wet tenacities of 2.73 grams per denier and 1.68 grams per denier, respectively, as well as dry and wet elongations of 13.7% and 12.6% respectively. The apparent change in physical properties is caused mainly by shrinkage of the yarn with consequent proportional increase in yarn denier.

#### Example II

Viscose is passed through a spinneret containing 100 holes, with an average viscose delivery of 11 grams per minute, into an aqueous spinning bath containing 11% sulfuric acid, 23% sodium sulfate, 4% glucose and 0.7% zinc sulfate, said bath being maintained at 45° ± 1° C. The extruded filaments are guided through the bath by a plurality of roller guides selected to impose a tension on the yarn during a bath travel of 130 inches. The yarn is then led over a freely rotating transfer roller into a secondary bath, which

consists of an aqueous solution containing 2% sulfuric acid, maintained at  $92^{\circ}\pm 2^{\circ}$  C. through which it is guided by a plurality of roller guides, also designed to impose tension on the yarn, for a bath travel of 20 inches. From the secondary bath the yarn is led to a positively driven feed wheel, whence it is collected in a centrifugal bucket rotating at 10,000 R. P. M. in the usual way. The spinning speed (feed wheel speed) is 3600 inches per minute and the roller guides in the baths are such that a spin tension of 85 grams is obtained when the transfer roll runs at a peripheral speed of 2710 inches per minute. The finished yarn, washed and dried in the cake without bleaching, has a denier of about 100, (one denier per filament) a dry tenacity of 2.96 grams per denier, and a wet tenacity of 1.95 grams per denier with dry and wet elongations of 14.9% and 15.3% respectively.

By reference to the above examples, it will be apparent that yarn of exceptionally fine denier can be produced from viscose with great ease even though very high spinning speeds are employed. Yarn produced in accordance with the present invention will have a high tenacity and may therefore be used to great advantage in the production of sheer knit goods and light-weight woven fabrics. The quality of the yarn is vastly superior to that of fine denier viscose rayon produced in prior art processes in respect to yarn degradation, yarn tenacity and fineness of denier. The reason for this lies in the fact that the yarn denier can be reduced by a stretching operation in which much greater stretch can be secured than when stretching in the spinning bath is relied upon. The amount of stretch given the yarn affects in large measure the tenacity and denier of the final product; however, the stretch must be imposed on the yarn during a comparatively short period so as to prevent yarn degradation. If material yarn degradation takes place the tenacity of the yarn will be substantially lowered.

The composition of the hot acid stretching bath may be the same as that of the coagulating and regenerating bath with the attendant advantages of simplified bath make-up systems, use of hot bath overflow to maintain spinning bath temperature and composition, economical use ultimately as spinning bath, and the like. However, if high salt concentrations are used, the tendency toward crystallization in the hot acid stretching bath is increased so that it is frequently preferable to use a different hot bath composition. To this end then, compositions containing 2% to 13% sulfuric acid, 0 to 30% sodium sulfate and with or without zinc sulfate or glucose may be used. Inasmuch as the higher temperature of the secondary bath is conducive to carbonization of glucose, a glucose-free bath may be preferred. Inasmuch as greater stretch can be secured when the acid concentration in the hot acid bath is low, it is advantageous to keep the acid concentration in this bath at a low level, for example, 2% to 10%, when spinning fine denier filaments.

The temperature of the spinning bath is usually selected in the range of  $40^{\circ}$ – $50^{\circ}$  C., preferably  $45^{\circ}$ – $50^{\circ}$  C., as generally accepted in the art. The temperature of the secondary bath is selected in the range of  $60^{\circ}$  C. to boiling temperature, and usually  $90^{\circ}$ – $100^{\circ}$  C. This preferred range generally yields higher breaking tensions, that is, the tension to which a thread can be subjected before breaking.

The amount of tension imposed on the yarn in the spinning bath controls to a considerable extent the amount of stretch which can later be given the yarn in the hot acid bath. This relationship is qualitatively expressed in the following table in which the tension is measured on the yarn as it leaves the spinning bath:

| 10                   | Tension  | Breaking stretch |
|----------------------|----------|------------------|
|                      | Per cent |                  |
| 0.1 gram per denier  | 75       |                  |
| 0.4 grams per denier | 35       |                  |
| 0.5 grams per denier | 23       |                  |
| 0.9 grams per denier | 19       |                  |

Thus it is readily apparent that since a relatively large amount of stretch is essential when fine denier filaments are to be made, it is advantageous to keep the tension on the yarn in the spinning bath at a low level. The tension on the yarn in the spinning bath must be maintained below 1.0 gram per denier, and to obtain full advantage of the present invention the tension in the said spinning bath should not exceed 0.5 gram per denier.

By the process of the present invention it is practical to spin a yarn of 0.5 to 0.75 denier per filament at high speed while still keeping the yarn speed in the coagulating and regenerating bath sufficiently low to prevent entrance of this bath into the spinneret, which will result in plugged spinneret holes. As a consequence spinnerets of larger hole sizes can be used than has been possible in prior art processes.

The ratio of spinning speed to average linear viscose delivery speed for a viscose containing about 7% cellulose varies from about 1.45 for a 6.25 denier per filament yarn to about 3 for a one denier per filament yarn (1 D/F). The latter ratio is obtained by using a spinneret having holes about 0.0025 inch in diameter which is about the minimum hole size compatible with efficient spinning. To spin a 0.5 D/F yarn with such a spinneret will require a ratio of spinning speed to viscose delivery of about 6 which is considerably higher than can be tolerated by the prior art spinning processes. However, the present invention will permit ratios of 6 or higher by virtue of a 30%–60% or higher stretch imposed on the yarn during its passage through the bath by virtue of the hot treatment under tension which in turn allows for slower yarn speeds in the spinning bath than can be possible in the absence of the hot bath treatment.

The advantages of the foregoing can be appreciated by the following. In spinning fine denier per filament yarn the ratio of yarn speed, at a point, say, 25 inches from the spinneret, to viscose delivery is critical. For producing 1 D/F yarn by a single bath process this ratio is about 2.5 when a spinneret having holes about 0.0025 inch in diameter is used. Any decrease in filament denier without change in hole size will raise this ratio proportionately so that it will be about 5 for a 0.5 D/F yarn. By the process of this invention the ratio can be kept well below 5 or in the range 2.9 to about 4. Similarly, for a yarn of 1 D/F, this invention makes it possible to keep the ratio well below 2.5 or in the range 1.5 to about 2. These lower ratios are valuable in producing higher quality yarns by an economical procedure.

Since it is obvious that many changes and

modifications can be made in the details of the invention above described, it is to be understood that the invention is not to be limited except as set forth in the appended claims.

I claim:

1. The process of spinning regenerated cellulose yarn comprising filaments having a denier of less than one which comprises extruding a viscose solution into a coagulating and regenerating bath of the dilute acid type (of the order of 9% to 11% acid) with a ratio of yarn speed, at a point 25 inches from the spinneret, to viscose delivery speed of 2.9 to 4 (based on a 0.5 denier per filament yarn) to form yarns, maintaining said yarn under tension of less than 1 gram per denier during its passage through said coagulating and regenerating bath, removing said yarns from said bath and passing them, for a distance not to exceed 45 inches, based on a spinning speed of 3000 to 8000 inches per minute, through a 2% to 13% sulfuric acid bath having a temperature of 60° C. to boiling temperature, and stretching said yarns at least 30% to materially reduce their denier during their passage through said hot acid bath.

2. The process of spinning regenerated cellulose yarn comprising filaments having a denier of less than one which comprises extruding a viscose solution into a coagulating and regenerating bath of the dilute acid type (of the order of 9% to 11% acid) with a ratio of yarn speed, at a point 25 inches from the spinneret, to viscose delivery speed of 2.9 to 4 (based on a 0.5 denier per filament yarn) to form yarns, maintaining said yarn under tension of less than 1 gram per denier during its passage through said coagulating and regenerating bath, removing said yarns from said bath and passing them, for a distance not to exceed 45 inches, based on a spinning speed of 3000 to 8000 inches per minute, through a 2% to 13% sulfuric acid bath of a composition essentially the same as said coagulating and regenerating bath and having a temperature of 60° C. to boiling temperature, and stretching said yarns at least 30% to materially reduce their denier during their passage through said hot acid bath.

EMERSON A. TIPPETTS.